# EUROPEAN PATENT SPECIFICATION

(11) **EP 0 980 077 B1**
(45) Date of publication and mention of the grant of the patent: **19.03.2003**
(21) Application number: 99500116.1
(22) Date of filing: 09.07.1999
(51) Int. Cl.: G21G 4/06

(54) **Procedure for the incorporation of hazardous or costly substances onto aluminium supports with very low thickness of anodising**
Verfahren zum Einbauen von gefährlichen und teueren Stoffen auf Aluminiumträger mit einer sehr niedrigen anodisierten Stärke
Procédé d'incorporation de substances dangereuses ou coûteuses sur des supports en aluminium présentant une couche d'anodisation trés mince

(30) Priority: 10.08.1998 ES 9801720
(43) Date of publication of application: 16.02.2000
(73) Proprietor: CENTRO DE INVESTIGACIONES ENERGETICAS MEDIOAMBIENTALES Y TECNOLOGICAS (C.I.E.M.A.T.), E-28040 Madrid (ES)
(72) Inventor: Gascon Murillo, Jose Luis D., 28040 Madrid (ES)
(74) Representative: Del Santo Abril, Natividad

(56) References cited:
- EP-A- 0 015 807
- GARCIA-TORANO E ET AL: "Preparation and standardization of large-area sources for calibration of alpha-particle contamination monitors" NUCLEAR INSTRUMENTS & METHODS IN PHYSICS RESEARCH, SECTION - A: ACCELERATORS, SPECTROMETERS, DETECTORS AND ASSOCIATED EQUIPMENT, vol. 396, no. 1-2, 1 September 1997 (1997-09-01), page 130-134 XP004097889 ISSN: 0168-9002
- LALLY ET AL. : "Source preparation in alpha spectrometry" NUCLEAR INSTRUMENTS AND METHODS., vol. 223, 1984, pages 259-265, XP002121026 NORTH-HOLLAND PUBLISHING COMPANY. AMSTERDAM., NL
- FUSCHINI ET AL.: "A new method for preparing radioactive sources" NUCLEAR INSTRUMENTS AND METHODS., vol. 26, no. 2, March 1964 (1964-03), pages 301-304, XP002121134 NORTH-HOLLAND PUBLISHING COMPANY. AMSTERDAM., NL
- PATENT ABSTRACTS OF JAPAN vol. 013, no. 189 (M-821), 8 May 1989 (1989-05-08) & JP 01 014090 A (FUJI PHOTO FILM CO LTD), 18 January 1989 (1989-01-18)

## Description

The subject matter of the present invention is a procedure to deposit hazardous or costly substances onto the anodised layer of an aluminium support.

The applications of the subject matter of the invention are, mainly the preparation of extensive radioactive sources and in general the deposit onto anodised aluminium supports of hazardous (radioactive, toxic, medical, etc.) or costly products (silver salts for photography, noble elements for decoration, antithermal ceramic elements, etc.)

The Spanish standard UNE 21-72-90 and international one ISO 8769 specify the characteristics that radioactive sources used for the calibration of superficial contamination monitors must fulfil. According to this standard, the area of the radioactive source must have a surface of at least 100 cm² and, as to the homogeneity or distribution of the activity of the radionuclide on the source, there should not be a variation above 10% in the specific surface activity measured at different parts of the source.

The preparation of radioactive sources of large superficial area cannot be done with the electroplatting methods used in the preparation of small sources (less than 5 cm²) due to the problems that appear on the homogeneity of the electrical fields applied which give rise to an irregular distribution of the activity of the radionuclide on the surface, which causes a series of dark spots that deteriorate the appearance of the mentioned source.

An alternative to the electroplatting methods are the methods of direct platting of the solution of the radionuclide onto the support of the source as described in Lally et al. Nucl. Instr. Meth. 223 (1984)

259. Among these methods, the simplest one is the one consisting in the evaporation of the solution deposited on the support. The homogeneity of the activity on the surface of the source is quite acceptable, but has the drawback that the deposit is unprotected and may readily come off.

The procedure of the invention is based on the direct platting of the radionuclide solution onto an anodised aluminium support. The radionuclide, being absorbed onto the aluminium oxide porous layer, is platted in a homogeneous way and protected.

Conventional procedures for the incorporation of stable elements (Co, Mn, Cr, etc.) onto an anodised aluminium layer are well known, and are based on the use of aqueous solutions of the elements to be incorporated under diverse conditions of temperature, pH, concentration, etc.

The application of the above mentioned procedures to the preparation of extensive radioactive sources has not produced good results, obtaining very low yields (around 2%) for the deposit of the radionuclides. Besides, as a consequence of other stable elements being incorporated to the deposit, causes an increase in the thickness of the latter which degrades the radiation energy, making more difficult the calibration of the source.

The possible causes that may produce these poor results, are thought to be:
a) The thickness of the anodised aluminium layer of the supports of the extensive radioactive sources must be at most 4 µm, so that there is no important degradation in the radiation energy, much thinner, therefore, than the minimum 10 µm used in conventional anodising procedures.
b) Conventional procedures use stable element solutions, whose concentrations are in the 10⁻¹ M range, much above those of the radionuclide which are 10⁻¹⁰ M. The concentrations of the radionuclide cannot be in the same range as those of the stable elements due to the problems that working with very high radioactive activities would originate.

The process for the incorporation of the radionuclide to the aluminium oxide layer is ruled by the superficial liquid-solid interaction. It is this interaction that controls the solution volume absorbed and, therefore, the amount of radionuclide that deposits onto the porous aluminium oxide layer.

The procedure subject matter of the invention manages to increase this volume by modifying the surface tension between the liquid-solid phases; i.e., by varying the composition of the radionuclide solution it is possible to obtain a better absorption onto the anodised porous layer.

In order not to hinder the calibration of the source, it is necessary to limit to the maximum the contamination of the anodised layer, and thus it is essential to operate with a low solid residue rate.

On the other hand, a high steam pressure will allow to operate at room temperature which, besides providing easiness and economy, makes possible the platting of substances which would not endure high temperatures.

A series of tests were carried out with solutions of a radionuclide with different composition and surface tension values, and it was found that when the surface tension value was 72 din cm⁻¹ (versus air and at 20°C) very low yields were obtained (around 2%), whilst when the surface tension value was around 20 din cm⁻¹ (versus air and at 20°C) the yield was excellent (around 80%).

The procedure for the incorporation of hazardous or costly substances onto an anodised aluminium support subject matter of the invention consists in the use of solutions with small surface tension values (around 20 din cm⁻¹ versus air and at 20°C) in solutions which must present determined characteristics. Components
- The substance to be incorporated; which must be soluble in the solvent which accompanies it.
- A solvent which has a low residue rate.
- Various additives; in order to obtain the adequate surface tension and steam pressure values, in such a way that it is not necessary to use high temperatures.

### Parameters

- Surface tension; less than 25 din cm⁻¹ versus air and at 20°C
- Steam pressure; greater than 40 mm of Hg at 20°C
- Solid residue; less than 4.5 10⁻³ g/l

In order to help to a better understanding of the invention, a detailed description of a preferred embodiment will follow, with an orienting and not limiting character, supported by the figure attached, being an integral part of this descriptive report and which represents the incorporation yield of a 10⁻¹⁰ M solution of ²⁴¹Am onto an aluminium plate with an anodised thickness of 4 µm as a function of surface tension of the water-ethanol mixture used in the solution.

The reckoning of the deposit yield of the 10⁻¹⁰ M solution of ²⁴¹Am was done in the following way: Preparation of a sample with a solution volume which is a function of the plate surface, as will be stated below. Measurement of the radioactive activity.

Preparation of a solution volume identical to the preceding one and deposition of the same onto the anodised aluminium plate in the conditions that will be described below. Measurement of the radioactive activity of the anodised aluminium plate impregnated in this manner.$\text{R =} \frac{\text{Activity of the anodised aluminium plate}}{\text{Activity of the solution sample}} \text{x 100}$

The procedure for the preparation of extensive radioactive sources comprises the following stages:
A solvent - additive mixture is prepared that complies to the following conditions: surface tension below 25 din cm⁻¹, steam pressure greater than 40 mm of Hg at 20°C and solid residue below 4.5 10⁻³ g/l which in this case will be made up of a water ethanol mixture with a considerable larger rate of this latter product in a proportion at least of approximately 20/80.

The 10⁻¹⁰ M solution of the radionuclide is prepared with the previously prepared mixture from a solution of ²⁴¹Am in 4M nitric acid, by drying and change of medium.

The solution thus prepared is deposited by successive drops onto an aluminium support with a thickness of anodising of 4 µm. A volume of 1 ml is sufficient for one plate of 100 cm².

The excess is removed after one minute, by means of blotting paper.

The deposit which may have remained on the anodised layer is removed by rubbing with paper soaked in the solvent - additive mixture used for the dissolution of the radionuclide.

Once the example of a preferred embodiment of the invention has been described, the generalisation of the procedure for the incorporation of other substances onto anodised plates will be evident for any person skilled in the art.

The solvent shall be chosen as a function of the substance that is to be incorporated. Given that the solution thus prepared will not comply, in general, to the limits established for the surface tension, steam pressure and solid residue parameters which ensure the success of the procedure, it will be necessary to include surfactant additives which must also be compatible, in terms of solubility, with the solvent used.

The last removal stage, by rubbing, of the deposit which could have remained on the anodised layer, is essential in the application of the procedure to the preparation of extensive radioactive sources, in order to ensure the homogeneity of the radioactive activity and its endurance against mechanical aggressions, but may not be essential in other applications.

As regards the industrial performance of the procedure subject matter of the invention, it will be evident for any person skilled in the art that the removal of the excess solution by means of blotting paper is an operation whose purpose is the same as the high steam pressure requirement. Thus, for the performance of the method by hand, it will be possible to operate with a lower steam pressure as a function of the ability of the operator with the blotting paper, whilst in a mechanised production installation, it will be mandatory to respect the steam pressure values specified and simplify or even leave out the stage of removal of the excess by means of blotting paper.

## Claims

1. Procedure for the incorporation of hazardous or costly substances onto aluminium supports with very low thickness of anodising, **characterised in that** it comprises the following stages:
preparation of a solvent-additive mixture which complies to the conditions: surface tension below 25 din cm⁻¹, steam pressure greater than 40 mm of Hg at 20°C and solid residue below 4.5 10⁻³ g/l,
preparation of a 10⁻¹⁰ M solution of the substance to be incorporated with the mentioned solvent - additive mixture,
deposition of the solution thus prepared by successive drops onto an aluminium support with an thickness of anodising of 4 µm,
removal of the excess, after one minute, by means of blotting paper,
removal of the deposit which may have remained on the anodised layer by rubbing with paper soaked in the solvent - additive mixture mentioned before.

2. Procedure for the incorporation of hazardous or costly substances onto aluminium supports with very low thickness of anodising, according to claim 1, **characterised in that** the substance to be incorporated mentioned is a radionuclide, preferably ²⁴¹Am, and the solvent - additive mixture is made up of water and ethanol.

## Patentansprüche

1. Verfahren zum Einbau gefährlicher oder hochwertiger Substanzen auf Aluminiumträgern mit sehr dünner eloxierter Schicht, **dadurch gekennzeichnet, dass** aus folgenden Phasen besteht:
Zubereitung einer Mischung aus Zusatzstoff und Lösungsmittel, welche die Bedingungen erfüllt, eine Oberflächenspannung von kleiner 25 din/cm⁻1, einen Dampfdruck von größer 40 mm Hg bei 20°C und festen Rückstand von weniger als 4,5 10⁻³ g/l zu besitzen,
Zubereitung einer M 10⁻¹⁰- Lösung der Substanz, die zusammen mit der genannten Mischung aus Wirkstoff und Lösungsmittel eingebaut wird,
Applikation der auf diese Weise zubereiteten Lösung in aufeinanderfolgenden Tropfen auf einem Aluminiumträger mit 4 µm starker eloxierter Schicht, nach einer Minute Entfernung des Überschusses mittels Löschpapier,
Entfernung der Ablagerung, die möglicherweise auf der eloxierten Schicht zurückgeblieben ist, durch Abreiben mit Papier, das mit der zuvor genannten Mischung aus Zusatzstoff und Lösungsmittel getränkt wurde.

2. Verfahren zum Einbau gefährlicher oder hochwertiger Substanzen auf Aluminiumträgern mit sehr dünner eloxierter Schicht gemäß Anspruch 1, **dadurch gekennzeichnet, dass** die genannte einzubauende Substanz ein Radionuklid ist, vorzugsweise ein ²⁴¹Am, und dass sich die Mischung aus Zusatzstoff und Lösungsmittel aus Wasser und Ethanol zusammensetzt.

## Revendications

1. Procédé pour incorporer des substances dangereuses ou de coûts élevés dans des supports en aluminium d'une très faible épaisseur anodisée, **caractérisé en ce qu'**il comprend les phases suivantes :
préparation d'un mélange d'additif et de dissolvant conforme aux conditions de tension superficielle situées en dessous de 25 din/cm⁻¹, de pression de vapeur supérieure à 40 mm de Hg à une température de 20° C et un résidu solide en dessous de 4,5 10⁻³ g/l,
préparation d'une solution M 10⁻¹⁰ de la substance qui va s'incorporer au mélange d'additif et de dissolvant antérieurement mentionné,
déposition de la solution ainsi préparée par gouttes successives sur un support en aluminium d'une épaisseur anodisée de 4 µm,
élimination de l'excédent, après un délai d'une minute, avec du papier buvard,
élimination de l'éventuel dépôt sur la tôle anodisée en frottant avec le papier imprégné du mélange d'additif et de dissolvant mentionné antérieurement.

2. Procédé pour l'incorporation de substances dangereuses ou de coût élevé sur des supports en aluminium d'une très faible épaisseur anodisée, selon la revendication 1, **caractérisé en ce que** la substance mentionnée que va s'incorporer est un radionucléide, préférentiellement un ²⁴¹Am, et le mélange d'additif et de dissolvant se compose d'eau et d'éthanol.
